

H. C. PRITHAM.

PAPER TUBE AND PROCESS OF WATERPROOFING THE SAME.

APPLICATION FILED MAY 28, 1914.

1,174,279.

Patented Mar. 7, 1916.



WITNESSES:

H. W. Meade  
E. M. Culver.

INVENTOR

Henry C. Pritham  
BY  
A. M. Wooster  
ATTORNEY

# UNITED STATES PATENT OFFICE.

HENRY C. PRITHAM, OF BRIDGEPORT, CONNECTICUT, ASSIGNOR TO UNION METALLIC CARTRIDGE COMPANY, OF BRIDGEPORT, CONNECTICUT, A CORPORATION OF CONNECTICUT.

## PAPER TUBE AND PROCESS OF WATERPROOFING THE SAME.

1,174,279.

Specification of Letters Patent.

Patented Mar. 7, 1916.

Application filed May 28, 1914. Serial No. 841,494.

*To all whom it may concern:*

Be it known that I, HENRY C. PRITHAM, a citizen of the United States, residing at Bridgeport, county of Fairfield, State of Connecticut, have invented an Improvement 5 in Paper Tubes and Processes of Waterproofing the Same, of which the following is a specification.

In the accompanying drawing forming a 10 portion of this specification, the figure is a representation of a paper tube in perspective.

In the production of paper tubes, especially tubes which are adapted for use in 15 the manufacture of bodies for paper cartridge shells, it is always desirable and frequently necessary that the tubes shall be of uniform diameter throughout; shall present a smooth and even surface; that the tube 20 shall be waterproof, and also, in order to make it a salable and attractive article, that the color shall appear the same, or substantially the same, over the entire outer surface of the tube.

25 The object of the present invention is to produce such a tube, and by employing the process hereinafter set forth, such object is accomplished.

Paper tubes are usually made by rolling a 30 sheet of paper into tubular form and sticking the same, so that it retains its tubular shape. In order that this may be easily accomplished, paper intended to be made into tubes is usually made uncalendered or 35 nearly so. It will be seen that such tubes will be very sensitive to atmospheric conditions, absorbing water easily, and changing their diameters according to the amounts of water absorbed. In order to prevent this,

40 such paper tubes are usually first brought to exact size by being passed through a suitable sizing die, which also tends to put a certain amount of polish upon the tubes, after which they are immersed in a bath of 45 molten paraffin wax or a mixture thereof.

One disadvantage of such treatment lies in the fact that it is necessary to impregnate the tube with a large percentage of such 50 waterproofing material. The paper tubes made in this way are never evenly absorbent at different parts and the waterproofing material is not evenly distributed throughout the tube. This renders the tubes, especially

in the case of colored tubes, more or less translucent at different places, and hence 55 blotchy or mottled.

I have found by repeated experiments that paper tubes treated by impregnating or coating with a small percentage of a polymerizable oil or a solution thereof in molten 60 wax, and in which the polymerizable oil is thereafter gelatinized by any suitable means, are waterproofed in a superior manner and do not show the mottling or blotching usually found. A composition preferably em- 65 ployed for such waterproofing purposes consists of tung oil, otherwise known as Chinese wood oil, dissolved in molten paraffin wax in proportions of three parts of oil to ninety-seven parts of molten paraffin wax. 70 It should, however, be understood that my invention is not limited to the specific use of Chinese wood oil dissolved in paraffin wax, but other polymerizable oils may be used, and the composition of the water- 75 proofing and the proportions of the ingredients may be varied to suit special requirements without exceeding the scope of this invention. Tubes, so waterproofed, are heated to a higher temperature than that 80 of the bath in order to drain off the excess of wax and thoroughly polymerize and gelatinize the oil contained therein.

By employing tung oil, or its equivalent, dissolved in paraffin wax, the waterproofing 85 material is not only caused to fill the interstices between the fibers of the paper, but also actually fills the capillary openings in said fibers.

Having thus described my invention, I 90 claim:

1. The process of waterproofing paper tubes for cartridge shell bodies which consists in impregnating the tubes with a solution of a polymerizable oil in a molten wax 95 which possesses lubricating qualities, and thereafter heating the tubes in order to gelatinize the absorbed polymerizable oil.

2. The process of waterproofing paper tubes for cartridge shell bodies which consists in impregnating the tubes with a solution of Chinese wood oil in a wax which possesses lubricating qualities, and thereafter heating the tubes in order to gelatinize the oil contained therein. 100

3. The process of waterproofing paper

tubes for cartridge shell bodies which consists in impregnating the paper tubes with a solution consisting of three parts Chinese wood oil in ninety-seven parts of paraffin wax, and thereafter gelatinizing the Chinese wood oil contained therein.

4. As a new article of manufacture, a paper tube for cartridge shell bodies waterproofed with a polymerizable oil and a wax which will act as a lubricant, the polymerizable oil being gelatinized therein.

5. As a new article of manufacture, a paper tube for cartridge shell bodies waterproofed with Chinese wood oil and paraffin

wax, the Chinese wood oil being gelatinized therein.

6. As a new article of manufacture, a paper tube for cartridge shell bodies having a waterproof coating, the coating consisting of and being in the proportion of three parts of Chinese wood oil to ninety-seven parts of paraffin wax.

In testimony whereof I affix my signature in presence of two witnesses.

HENRY C. PRITHAM.

Witnesses:

CHARLES F. LINDSAY,  
MARY S. BURROUGHS.